

A. C. L. EKSTRÖM.  
COMBUSTION OF WASTE FUELS.  
APPLICATION FILED AUG. 6, 1918.

1,295,455.

Patented Feb. 25, 1919.



Fig. 1.



Fig. 2.



Fig. 4.



Fig. 3.

Inventor  
A. C. L. Ekström

By his Attorneys

Pennie Davis Marvin & Edmunds

# UNITED STATES PATENT OFFICE.

AXEL C. L. EKSTRÖM, OF BALLSTON SPA, NEW YORK.

## COMBUSTION OF WASTE FUELS.

1,295,455.

Specification of Letters Patent. Patented Feb. 25, 1919.

Application filed August 6, 1918. Serial No. 248,633.

*To all whom it may concern:*

Be it known that I, AXEL C. L. EKSTRÖM, a citizen of the United States, residing at Ballston Spa, in the county of Saratoga, 5 State of New York, have invented certain new and useful Improvements in the Combustion of Waste Fuels; and I do hereby declare the following to be a full, clear, and exact description of the invention, such as 10 will enable others skilled in the art to which it appertains to make and use the same.

The present invention has for its object to mix and burn waste fuels, whose combustion individually, is impracticable, so that, by 15 the practice of the invention a low cost fuel is obtained that may be economically burned, as hereinafter described, although its constituent ingredients, by themselves, are recognized as being incapable of successful use 20 as a fuel by any usual or ordinary method of combustion.

At every locomotive cleaning pit or ash dump, or where wastefully operated boilers are in operation, a large tonnage of refuse, 25 containing a high percentage of combustible material is available in the form of unburned bituminous coal, or coke, or anthracite coal but partly burned. When this combustible material is screened out, by either 30 the wet or dry process, it will not make a successful fuel capable of carrying a sustained fire, because of its inherent clinkering characteristic, resulting in a spotty fire indicating that the combustion is not complete. 35 The incompleteness of the combustion is due to the clinkering referred to which tends to close up the fuel bed, depriving it of its open character and correspondingly preventing successful combustion. Similar clinkering 40 characteristics are likewise inherent in other bituminous fuel wastes, such as coke oven screenings, the product known as coke breeze. In so far as I am aware, it has been heretofore found impracticable to utilize the waste 45 products referred to for the production of a satisfactory boiler fuel.

At every anthracite mine, after all of the prepared sizes have been taken out, and after all of the regular commercial steam sizes 50 have been taken out, there is a large waste tonnage (so-called slush) which is carried off from the property in liquid shape, but which carries as high as 60% of solids when the slush is passed through a screen of 55 3/64ths inch mesh. These solids contain a

large percentage of useful combustible material, after the water has been drained out. The solids obtained are in the shape of coal dust mixed with clay and other impurities. It is impracticable to use it alone upon a 60 boiler fuel bed for the reason that the individual particles are so light that with the employment of the usual forced draft, the particles will to a very large extent pass through the boiler flues before combustion 65 has taken place.

I have discovered that by appropriately combining the ash waste or coke oven waste above referred to with the mine waste described, a composite fuel is obtained of such 70 a character that it can be burned to great advantage as a boiler fuel, when the respective wastes are combined in such proportions as to not only obviate their individual deficiencies for boiler firing, but even to utilize 75 said individual deficiencies for the purpose of mutually correcting or compensating for each other. Thus, the clinkering characteristic of the ash waste or coke breeze is made available to serve as a binder for the light 80 particles of the anthracite mine waste, whereas the higher percentage of carbon present in the anthracite mine waste so raises the total carbon content of the mixture as to permit obtaining the required heat units per 85 volume of the composite mixture.

In practice, I employ from 10 to 20% of the bituminous ash wastes to 90 to 80% of the anthracite mine wastes. As noted, the main function of the ash waste is to serve 90 as a binder for the anthracite mine waste, and the relative percentages of the two kinds of wastes making up the composite fuel will at all times be so adjusted as to supply the more or less varying requirements of the 95 binding materials necessary to hold the dust containing the higher per cent. of carbon in position until the combustion has taken place.

In the accompanying drawing, I have 100 indicated a form of grate-bar of a type that I have found fully adapted to the successful combustion of the composite fuel described.

In said drawing:

Figure 1 represents, in side elevation, a 105 general view of a grate made up of a series of said grate-bars and their supports;

Fig. 2 represents a top plan view of an intermediate member of the series;

Fig. 3 represents a section on the line 3—3 110

of Fig. 2; and Fig. 4 is a section on the line 4—4.

Referring to the drawing, it may be noted that grate-bars are provided with a series 5 of slots  $\alpha$ . These slots should preferably be 1/16 of an inch wide, and not more than 5/64 of an inch wide at their upper plane, and should widen downwardly, as shown,—the object being to have the slots sufficiently 10 small to permit the bar to support the fuel mechanically and yet secure freedom from losses of coal through the bars, while at the same time giving them the necessary supply 15 of air to secure complete combustion, the furnace being otherwise of any suitable standard design utilizable with forced draft. The grate-bar shown in the drawing provides approximately 11% of air space, which is sufficient to pass the necessary supply of air

to obtain the practically complete combustion desired.

Having thus described my invention, what I claim is:

1. A composite fuel for steam boiler furnaces, comprising anthracite mine waste ad- 25 mixed with a clinkering ash waste of the kind described in such proportions that the ash waste will act as a binding agent to maintain the anthracite mine waste in position during the combustion of the composite 30 fuel; substantially as described.

2. A composite fuel for steam boiler furnaces, comprising from 80 to 90% of anthracite mine waste and 10 to 20% of clinkering ash waste; substantially as described. 35

In testimony whereof I affix my signature.

AXEL C. L. EKSTRÖM.

Copies of this patent may be obtained for five cents each, by addressing the "Commissioner of Patents.  
Washington, D. C."